

April 21, 1931.

F. B. BELL ET AL

1,801,994

PROCESS FOR MAKING HEAVY DUTY SPRINGS

Filed July 22, 1926

*Fig. 1*



*Fig. 2*



*Fig. 3*



*Inventor:*

Frank B. Bell & Oscar R. Wikander

*By: Munday, Clarke & Carpenter, Attys.*

## UNITED STATES PATENT OFFICE

FRANK B. BELL AND OSCAR R. WIKANDER, OF PITTSBURGH, PENNSYLVANIA, ASSIGNORS TO EDGEWATER STEEL COMPANY, OF PITTSBURGH, PENNSYLVANIA, A CORPORATION OF PENNSYLVANIA.

## PROCESS FOR MAKING HEAVY-DUTY SPRINGS

Application filed July 22, 1926. Serial No. 124,163.

This invention relates in general to the manufacture of heavy duty springs and a method of sizing the ring, and more particularly to heavy duty springs constructed of inner and outer members alternately arranged and provided with bevelled intervening faces operating through wedging action under compression of the spring to stretch and compress the material of the 10 rings and a method of sizing the rings so that they will permanently retain a given form and will not sag under operating strains or the like.

These springs rely upon the tensile strength 15 and compressive resistive strength for their spring action and this strength is increased upon stretching or compressing the material. It is a primary object of the present invention to provide a method of stretching and 20 compressing the material that will at the same time size the ring or form it to operating size after the spring elements have been fully formed and heat treated, to increase the strength and flexibility of the rings and 25 to prevent sagging of the spring in use.

Another important object of the invention is to provide a spring, the yielding movement of which is limited by the spring itself, and that when the maximum yield is reached the 30 spring forms a substantially solid column for supporting the load, and thus prevents overloading or injury such as may be caused by undue strains.

Numerous other objects and advantages of 35 the invention will be apparent as it is better understood from the following description, which, taken in connection with the accompanying drawings, discloses a preferred embodiment thereof.

Referring to the drawings,

Figure 1 is a section through a spring of the character above described; and

Figs. 2 and 3 are enlarged fragmentary sections showing the spring both free of and 45 under compression.

Our present invention does not relate to the method of forming the spring elements. The spring is, however, constructed of outer solid ring members 11 and inner solid ring members 12. The outer members are pro-

vided with internal bevelled or inclined faces 13 and the inner members are provided with companion bevelled or inclined faces 14. In the present instance a pair of beveled faces is provided on each ring element and these meet in a circumferential line extending about the largest diameter of the internal elements and the smaller diameter of the external.

Our present invention has for its purpose the provision of a method of sizing springs or 55 spring rings of this type, so that they will maintain a predetermined size throughout their period of service and to increase the elasticity or tensile strength of the ring. This is accomplished by forming the ring to a size slightly smaller than operating size 60 and stretching the ring when assembled, preferably between suitable dies, a predetermined number of times, such as by assembling an entire spring or taking each ring unit separately and between dies formed in accordance with the co-operating rings and applying a pressure to the dies or spring that is in excess of the maximum spring power. This pressure is preferably applied, released and 65 re-applied a multiple of times or until the desired condition is obtained. It will be understood, however, that under certain conditions it may not be desirable to treat all of the rings in this manner and that upon occasion any one or all of the outer rings may 70 be stretched or one or all of the inner rings may be compressed to accomplish a slightly different result.

When a die is used for stretching or compressing the rings, movement of the die is preferably limited so that an effect would be obtained similar to that which would be obtained if the rings were stretched while assembled; that is, when under full compression the adjacent surfaces of the outer rings, the inner rings, or both the outer and inner rings will be in contact, this being the limit of the movement of the spring. The pressure is applied until sufficient movement is obtained to cause a contact of the surfaces of adjacent rings at each application, and it will be noted that when so applied during the first application the ring or rings under treatment will be either stretched or compressed. During this first stretching or com-

55

60

65

70

75

80

85

90

95

100

pression, however, the strain on the fibres in the metal is not equal and by repeatedly applying a pressure the strain on the fibres in the metal is gradually equalized. This pressure should be repeatedly applied and released until the repetitions have amounted to some fifteen or twenty times, or until no more displacement of the fibres of the metal occurs, and the stretching or compressing of the metal is preferably carried to the extent of approximately one-third of one per cent. Since the strain of the ring and the strain on the fibres of the ring are equal or substantially so, when the ring is once stretched to size it will not sag under operating strains, as these are slightly less than the strain applied during the sizing process.

An important advantage flowing from this operation is that the pressure thus applied for a number of times bringing the inner rings into contact is greater than the force that the spring can receive in service. Stated differently, my improved process provides a test for the springs that insures against breakage up to full compression. It will, of course, be manifest that any pressure that will accomplish the result is contemplated within the spirit and scope of the invention.

It is thought that the invention and many of its attendant advantages will be understood from the foregoing without further description and it will be manifest that the process selected in connection with the description of the preferred embodiment may be departed from in various ways without departing from the spirit and scope of the invention.

We claim:

1. The process of making springs, which comprises providing a plurality of inner and outer solid rings adapted to be alternately arranged in a spring assembly, and provided with beveled faces for interengagement in such assembly, arranging said rings with the beveled faces in engagement and applying pressure thereto in controlled amount for increasing the elastic limit of the material.

2. The process of making springs, which comprises providing a plurality of inner and outer solid rings adapted to be alternately arranged in a spring assembly, and provided with beveled faces for interengagement in such assembly, arranging said rings with the beveled faces in engagement and applying pressure thereto in sufficient amount to increase the elastic limit of the material.

3. The process of making springs, which comprises providing a plurality of inner and outer solid rings adapted to be alternately arranged in a spring assembly, and provided with beveled faces for interengagement in such assembly, arranging said rings with the beveled faces in engagement and applying pressure thereto under controlled conditions

for increasing the elastic limit of the material.

4. The process of making springs, which comprises providing a plurality of inner and outer solid rings adapted to be alternately arranged in a spring assembly, and provided with beveled faces for interengagement in such assembly, arranging said rings with the beveled faces in engagement and applying pressure thereto in amount greater than the spring will sustain in service.

5. The process of making springs, which comprises providing a plurality of inner and outer solid rings adapted to be alternately arranged in a spring assembly, and provided with beveled faces for interengagement in such assembly, arranging said rings with the beveled faces in engagement and repeatedly applying pressure thereto to increase the elastic limit of material.

6. The process of making springs, which comprises providing a plurality of inner and outer solid rings adapted to be alternately arranged in a spring assembly, and provided with beveled faces for interengagement in such assembly, arranging said rings with the beveled faces in engagement and applying pressure thereto until rings of said spring assembly are in contact at faces other than said beveled faces, whereby the elastic limit of the material is increased.

7. The process of making springs, which comprises providing a set of outer solid rings and a set of inner solid rings, the members of said sets being adapted to be arranged to alternate with the members of the companion set, and the members of both sets having beveled faces for interengagement in assembly, and stretching the outer rings by pressure applied under controlled conditions to increase the elastic limit of the material.

8. The process of making springs, which comprises providing a plurality of inner and outer solid rings adapted to be alternately arranged in a spring assembly, and provided with beveled faces for interengagement in such assembly, arranging said rings with the beveled faces in engagement and repeatedly applying pressure thereto and under controlled conditions, said pressure being in excess of that the spring will sustain in service, whereby to wear in and smooth the engaging faces of the ring.

9. The process of making springs, which comprises providing a plurality of inner and outer solid rings adapted to be alternately arranged in a spring assembly, and provided with beveled faces for interengagement in such assembly, arranging said rings with the beveled faces in engagement and repeatedly applying pressure thereto and under controlled conditions.

FRANK B. BELL  
OSCAR R. WIKANDER.